

## UNITED STATES PATENT OFFICE.

ADDISON F. HOFFMAN, OF PITTSBURGH, PENNSYLVANIA.

## UTILIZATION OF CELLULOSE LIQUORS.

No Drawing.

Application filed April 1, 1919. Serial No. 286,740.

*To all whom it may concern:*

Be it known that I, ADDISON F. HOFFMAN, citizen of the United States, residing at Pittsburgh, in the county of Allegheny and State of Pennsylvania, have invented new and useful Improvements in the Utilization of Cellulose Liquors, of which the following is a specification.

The manufacture of pulp from wood is ordinarily carried out in this country, according to one of two principal processes, namely the sulfite process or the soda process. In relatively few pulp mills other digestive fluids are used for the production of pulp. The extract or residual liquid, obtained in the sulfite process, and commonly referred to in the art as "sulfite cellulose waste liquor," consists of an aqueous solution, strongly acid in reaction, containing salts of calcium and magnesium, and also containing lignone derivatives and also derivatives or compounds of resins, organic acids, starches, sugars, oils, tars, gums and perhaps other substances, the liquor in fact containing practically all of the original constituents of the wood, except the cellulose, although of course in the form of compounds of a very different nature than those contained in the original wood treated. The exact nature of this waste liquor also varies to some extent depending upon the particular kind of wood under treatment, spruce wood giving a liquor having substantially different properties in many respects, from the liquor obtained from poplar and other pulp woods.

The liquor obtained in the soda pulp process is of a substantially different character, although it also contains compounds or derivatives of many of the substances enumerated above. This liquor is also alkaline in reaction.

According to the preferred form of the present invention, I separate the pulp as completely as possible from the liquor or this operation is preferably effected by the pulp maker. I then add to the sulfite waste liquor, a sufficient amount of the soda pulp liquor to render the mixture neutral or slightly alkaline. Both of these liquors may vary considerably in concentration or density, but with liquors of ordinary concentration, say 8° to 10° Baumé, I find in some instances that one part of the soda liquor may be added to about three parts

of the sulfite waste liquor, with satisfactory results. It is not necessary, although advisable that the liquors be used in such relative proportions as to produce about the degree of alkalinity referred to in this example. The neutral liquor seems to be more advantageous in many cases, since it is substantially more stable, thereby producing less decomposition, both during the concentration operation, and while in storage after treatment. The neutralization produces a considerable amount of precipitate, which in many cases contains large quantities of neutral calcium sulfite or magnesium sulfite, which may be utilized for the preparation of bisulfite liquor, for paper or pulp making. The precipitate is preferably removed, for example by filtering or filter pressing, after which the remaining liquor is concentrated in suitable apparatus (vacuum apparatus being preferred) until a density of from 30° to 35° Baumé is obtained. The liquor may then again be filtered if desired, and is then ready to be run into receptacles for shipment. This concentrated liquor is quite stable, can be kept for long periods of time, and is readily transportable, readily miscible with water and non-inflammable.

This concentrated liquor has been found to give excellent results, when diluted and used in place of oil, as a lubricant for the cutting edges of tools used in metal cutting. The liquor in its concentrated form may be diluted with say 8 to 10 parts of water at the time of use, but these proportions can be varied widely, depending upon the particular conditions of use. The diluted liquor is found to be suitable for use in drilling, turning, thread cutting, milling, and various other operations in metal working. The liquor may be supplied to the cutting edge or cutting point of the tool in any suitable manner, and for the best results should be supplied freely, that is to say in such quantities that the end of the tool, and the work is kept thoroughly wet. As is the common practice in cutting metals, the liquor which drains away can be pumped up into the supply tank for reuse, as many times as desired.

The material has been found to be in some respects much superior to soda water, soapy water, oil emulsions and similar liquids heretofore largely employed, and moreover seems

to possess some point of advantage over the highly expensive lard oil previously in common use.

While I prefer to employ the acid pulp liquor and soda pulp liquor, I can use, although less advantageously, sulfite waste liquor neutralized with ordinary alkalies, for example soda, lime, magnesia, chalk, or magnesite. In some instances soda pulp liquor, without neutralization, or after substantially complete neutralization, the same may be employed. Neither of these two liquors seems to give as good results as those obtained when using the acid pulp liquor and the alkaline pulp liquor.

In some instances, other kinds of pulp liquor, such as those produced from the sodium sulfate pulp process, or the sodium sulfide pulp process may be used, but these are both inferior to the preferred forms of the invention.

The concentrated liquor, or the concentrated and diluted liquor may be used alone, or may be used in conjunction with other cutting compounds, whether solutions or emulsions.

In a modified form of carrying out the process, the sulfite pulp liquor in a substantially neutral state, and the soda pulp liquor in its original alkaline state may be separately concentrated, and the concentrated solutions mixed. This however is usually a more expensive procedure, and does not produce substantially better results, and in many cases does not produce results which are even as good as those produced in the preferred form of the process as above described, since there is more alteration in the colloidal content of the liquors, by evapo-

tion in a strongly acid or strongly alkaline condition.

What I claim is:

1. The herein described process of lubricating cutting tools, which comprises supplying thereto a lubricant liquor containing sulfite cellulose waste liquor.

2. The herein described process of lubricating cutting tools, which comprises supplying thereto a lubricant liquid containing a concentrate of sulfite cellulose waste liquor.

3. The herein described process of lubricating cutting tools, which comprises supplying thereto a lubricant liquor containing sulfite cellulose waste liquor rendered appreciably alkaline by the addition of soda pulp liquor.

4. A process of lubricating cutting tools which comprises supplying thereto, sulfite waste liquor having an alkaline material added thereto.

5. The hereinabove described process of lubricating cutting tools, which comprises supplying thereto a lubricant liquor containing waste liquor of wood pulp manufacture, at least partially neutralized.

6. A process of lubricating cutting tools, which comprises supplying thereto a lubricant liquor containing concentrated and re-diluted waste liquor of wood pulp manufacture, at least partially neutralized.

7. A process of lubricating cutting tools, which comprises supplying thereto a lubricant liquor containing concentrated waste liquor of wood pulp manufacture, at least partially neutralized.

In testimony whereof I affix my signature.

ADDISON F. HOFFMAN.